

## UNITED STATES PATENT OFFICE

FRITZ ROTHE, OF AACHEN, AND HANS BRENEK, OF PORZ, NEAR COLOGNE, GERMANY,  
ASSIGNORS TO RHENANIA VEREIN CHEMISCHES FABRIKEN A. G., OF COLOGNE, GERMANY

## PROCESS FOR TRANSFORMING THE BARIUM AND STRONTIUM SULPHATES

No Drawing. Application filed November 3, 1925, Serial No. 66,641, and in Germany November 12, 1924.

This invention relates to the transformation of alkaline earth metal sulphates into other alkaline earth metal compounds and more particularly to the transformation of barium and strontium sulphates.

The principal object of the invention is the provision of a method for transforming barium and strontium sulphates into desired compounds which is simpler than the known methods in that the intermediate reduction into the corresponding sulphides is eliminated. The said transformation is effected by mixing the sulphates with silica and heating to high temperatures in the presence 15 of steam.

The usual method of utilizing the barium- and strontium sulphates consists, as it is known, in transforming them by reduction with coal into the corresponding sulfides from 20 which the carbonates, chlorides, nitrates, oxides, hydroxides etc. of said alkaline earth metals can be obtained in a known manner. In these processes hydrogen sulfide is always formed which is generally burnt in the Claus 25 furnace in order to obtain sulphur, as it is especially known in the case of barium sulfide.

Now it has been found that said alkaline earth sulphates can be transformed into other 30 alkaline earth compounds in a much simpler way and especially without the formation of sulfides as intermediate products, if the sulphates mixed with silica or materials very rich in silicic acid are heated up to high temperatures in the presence of steam preferably 35 in an oxidizing atmosphere. By this manner of operating the sulphur contained in the alkaline earth sulphates is directly obtained as sulfurous acid the further treatment of which 40 occurs in a known manner. The alkaline earth silicate obtained can be utilized in different ways. For instance it may be decomposed by an acid in order to obtain alkaline earth salts. In this case the silica may be 45 again introduced in the process to act upon the sulphates. It is especially advantageous to use the silica in such a quantity with respect to the alkaline earth sulphate that the alkaline earth silicates obtained are of a type 50 between  $\text{Me}_2\text{SiO}_4$  and  $\text{Me}_3\text{SiO}_5$ .

Under the influence of a treatment with water these alkaline earth silicates split up a part of their alkaline earth as alkaline earth hydroxide, the rest of the alkaline earth remaining bound to the silica as metasilicate. 55

For instance:



or



The metasilicate obtained is mixed with further quantities of alkaline earth sulphates, then the mixture is heated to incandescence, as described above, in the presence of steam. 65 By this process ortho- or trisilicate or intermediate products between these two silicates are formed again according to the proportion in which the alkaline earth silicate and the alkaline earth sulphate are mixed. This process corresponds for instance to the following 70 equation:



or



By this manner it is easily possible to obtain barium or strontium-hydroxides, which may either be used in their present state or 80 may be transformed into other barium- or strontium-compounds, for instance into carbonates, chlorides etc. without the necessity to remove the sulphuretted hydrogen, which is formed from the sulphide in the usual process. 85

The steam required for the reaction may be taken from a special source and mixed with the heating gases. But it is also possible to heat the furnaces in which the reaction is effected by a fuel very rich in hydrogen which 90 furnishes by its combustion large quantities of steam, as for instance oil, producer gas from lignites and others.

## Example

100 parts of a heavy spar containing 92.25% of  $\text{BaSO}_4$  and 7.01% of  $\text{SiO}_2$  are intimately mixed with 5 parts of sand containing 98.8% of  $\text{SiO}_2$  and heated to about 1200° 100 in a revolving furnace under simultaneous

introduction of steam, care being taken to maintain an oxidizing atmosphere in the inner furnace by introducing a sufficient quantity of air.

5 The final product leaving the furnace is extracted with water by which 36.8% of BaO is dissolved as bariumhydroxide. The final product contains 83.64% of BaO. As the mixture is chosen to form  $2\text{BaO}\cdot\text{SiO}_2$ , only 10 41.82% of BaO can be expected to be soluble in water. Thus the 36.8% of the soluble BaO obtained represents 88% of the theoretic yield.

We claim:

1. The process for transforming barium-15 and strontium-sulphates comprising mixing said sulphates with silica and heating said mixture in an oxidizing atmosphere and in the presence of steam to a temperature of at least 1100° C.

20 2. The process for transforming barium- and strontium sulphates comprising mixing said sulphates with silica and heating said mixture in an oxidizing atmosphere to a temperature of at least 1100° C. by the aid of 25 heating gases containing steam.

3. The process for transforming barium- and strontium-sulphates comprising mixing said sulphates with silica in such a proportion that silicates of a type between  $\text{Me}_2\text{SiO}_4$ , 30 and  $\text{Me}_3\text{SiO}_5$  are formed and heating said mixture in an oxidizing atmosphere and in the presence of steam to a temperature of at least 1100° C.

4. The process for transforming barium-35 and strontium-sulphates comprising mixing said sulphates with silica in such a proportion that silicates of a type between  $\text{Me}_2\text{SiO}_4$  and  $\text{Me}_3\text{SiO}_5$  are formed, heating said mixture in an oxidizing atmosphere and in the 40 presence of steam to a temperature of at least 1100° C., decomposing the alkaline earth silicates obtained by treatment with water into alkaline earth hydroxides and a residue insoluble in water consisting essentially of alkaline earth metasilicate and introducing said 45 silicate again in the process for reacting with the sulphates.

Dr. FRITZ ROTHE.  
Dr. HANS BRENEK.